

1,082,722.

D. B. W. ALEXANDER.  
METHOD OF CONSTRUCTING ROADWAYS.  
APPLICATION FILED APR. 9, 1912.

Patented Dec. 30, 1913



Fig. 2.



Fig. 3.



Witnesses.

C. R. Pollard

C. Severance

Inventor.  
D. Basil W. Alexander.

by

Howard Shouse  
Atty's.

# UNITED STATES PATENT OFFICE.

DANIEL BASIL W. ALEXANDER, OF LOS ANGELES, CALIFORNIA.

## METHOD OF CONSTRUCTING ROADWAYS.

1,082,722.

Specification of Letters Patent.

Patented Dec. 30, 1913.

Application filed April 9, 1912. Serial No. 689,452.

To all whom it may concern:

Be it known that I, DANIEL BASIL W. ALEXANDER, a citizen of the United States, residing at Los Angeles, in the county of Los Angeles and State of California, have invented new and useful Improvements in the Method of Constructing Roadways, of which the following is a specification.

This invention relates to a method of constructing roadways and it is an object of the invention to provide a roadway in which the body portion is made up of rock suitably treated for preventing its shifting, suitable filling means being provided in connection therewith, after which a wearing surface forming a smooth roadway is applied above the same.

It is a further object of the invention to construct a roadway by preparing grouting material with an adhesive coating, of material tending to prevent the shifting of the individual pieces and filling the space in said grouting with fine material of any sort, after which the bed thus formed is treated with oil, and a surfacing material placed above the same and further treated with oil.

In the accompanying drawing forming a part of this specification, Figure 1 is a cross sectional view of a road bed constructed in accordance with the present method. Fig. 2 is a fragmentary sectional view showing the edge portion of the roadway upon an enlarged scale. Fig. 3 is an enlarged sectional view through a group of the bed stones of the roadbed showing the coating applied thereto.

The details and features of the invention will now be more particularly described, reference being had to the said drawing in which 5 indicates the grouting or base rock of the roadbed formed in accordance with this method, 6 the finer filling placed with the rock, and 7 a layer of oil above the same, and 8 and 9 a surfacing material and surface coat of oil respectively.

In forming road beds heretofore where large crushed rock is used as the base strata or layer, and particularly in oiled roads, the large rock at the base of the composition is found to readily shift in use so as to permit the oiled surface above to sink at intervals and form ruts after being used awhile.

One of the important features of the present invention is to provide a basic portion of the roadbed with crushed rock which is treated with a suitable coating of material

adapted to prevent the pieces of rock from slipping and shifting in the road bed, and also to preserve the rock from disintegration.

It is preferable to treat the crushed rock with bituminous substance forming a bituminous coating as 10, clearly shown in Fig. 3. This bituminous substance or coating is applied to the crushed rock before it is spread upon the roadbed, the substance or coating being allowed to harden or dry upon the rock before placing it upon the road bed. The ground is prepared in the usual way to form a roadbed being leveled to a proper depth after which the crushed rock treated with the coating as above described is spread over the ground to a suitable depth. The interstices of the rock are then filled with a finely crushed material, as for instance crushed rock that will pass through a number four mesh screen; said filling being indicated at 6 in the drawing. This material and the crushed rock are well rolled to form a smooth compact base strata for the roadbed.

In actual practice the rock employed at the bottom of the roadbed is dipped or otherwise coated in bituminous material of a low penetration, say at a temperature of from 300° F. to 500° F. according to the size of the rock, permitting the materials to cool while in motion or cooling them in water. This coated rock is then used in different proportions instead of the rock ordinarily used in making an oiled roadway. The rock ordinarily used is uncoated and is found to disintegrate through the action of moisture penetrating the roadbed so that it is more liable to shift from position and produce an uneven roadbed than if it was preserved in its original hardness. The rock thus prepared will, when combined in proper proportions to give the most desirable amount or volume of spaces or voids, which are then filled with clean screenings which are thrown on top of the rolled rock bed and carefully swept in. The roadway is next oiled with a suitable road oil, or oil just light enough to penetrate between the interstices of the coated rock and screenings. This oil is preferably heated to about 250° F. and will sink slowly into, and tend to soften the bituminous coating of the rocks so that the cementing action is increased and the rock and screenings closely bound together to prevent shifting in the roadbed.

Sand, as shown and designated as 8 in dia-

gram, is then swept on top of the surface, and is thoroughly rolled in; and then another application of oil, designated 9 in the diagram, is applied upon the whole to complete the surface.

Instead of laying the materials for the roadbed as heretofore described, I may take the bitumen-coated graded rock and thoroughly mix the same with screenings and sand in proper proportions to fill the voids, after which the entire mass may be transported to the place where it is to be laid, and rolled in place to form the roadbed. This rolled surface is finally treated with oil. This oil will penetrate and soften the hard bitumen, or, as it is termed, will "raise the penetration" (consistency) of the bitumen, and assist in binding the mass together, forming substantially the same character of roadbed as in the preferred form. Also another alternative form may be used which consists in combining with the uncoated rock, rock screenings and sand incorporating therein the requisite amount of powdered bitumen, all of these materials being in an unheated condition. After thoroughly commingling or mixing the mass together it is transported to the place of use and rolled in place upon the roadbed, after which the heated hydrocarbon is applied to bind the mass together, raising the penetration and forming a roadbed of substantially the same characteristics as heretofore described.

A roadway thus constructed produces a roadbed in which the oil will penetrate the mass and combine with the hard bitumen and thus raising the penetration to any desired point, depending on the amount of oil used and its specific gravity. Conversely it is found that the gravity of the oil is lowered by the solution of the bitumen from the rock, to a point where it will better cement the screenings and sand in the voids. Traffic will improve the road and the heat of the sun will tend to draw the bitumen to the wearing surface of the screenings and sand which are otherwise primarily deficient therein.

A road bed constructed in accordance with this invention thus provides good roads for country and highway uses which are smooth, dustless, cheap in initial cost and

upkeep, and not raveled by the suction of automobile tires or shoved out of place by any passing traffic. In other words a bituminous macadam roadway is produced with all its advantages, and a roadway made which more than saves in the item of maintenance what may be added by the cost of the bitumen used.

What I claim is:

1. The method of producing roadways, comprising the coating of crushed rock of graded sizes with a hard bituminous material and then cooling the same, then applying the rock to the surface to be covered by a roadbed, then partially filling the voids with rock screenings, then applying heated oil to the mass and allowing it to penetrate therein to soften the hard and brittle bituminous coating of the rock so that a cementing action is obtained, then sanding and rolling the sand into the interstices of the mass, and finally oiling the surface.

2. The method of constructing bituminous macadam roadways, comprising the coating of graded rock with a hard bituminous material; then laying and rolling the crushed rock with rock screenings added to form the basis of a roadbed, then oiling the roadbed and permitting the oil to penetrate to the bituminous coverings of the rock and combining with said bitumen for the purpose of cementing the particles of the roadbed together, and then applying sand, and further oiling the roadbed to produce a smooth waterproof surface.

3. The method of constructing roadways, comprising the mixing of hard bitumen, graded rock, rock screenings and sand, then spreading the mixture upon the road bed and rolling the same, and finally spraying sufficient oil to the rolled mass to soften the hard bitumen and cement the rock, sand and screenings together to one homogeneous mass.

In witness that I claim the foregoing I have hereunto subscribed my name this 4th day of April, 1912.

D. BASIL W. ALEXANDER.

Witnesses:

EDMUND A. STRAUSE,  
EARLE R. POLLARD.